

1

2,863,764

## COATED MAGNESIUM IRON TREATMENT

Grant E. Spangler, Philadelphia, Pa., and James W. Estes, New Brunswick, N. J., assignors to Air Reduction Company, Incorporated, New York, N. Y., a corporation of New York

No Drawing. Application July 23, 1956  
Serial No. 599,289

11 Claims. (Cl. 75—130)

This invention relates to an improved method for producing nodular cast iron and to a new addition agent for use in such method. More particularly, the invention relates to an improved method for injecting a new magnesium-containing treating agent beneath the surface of molten ferrous metal to produce a cast iron with improved properties and characteristics and with its graphitic carbon particularly in nodular or spheroidal form.

It is common knowledge in the art that cast irons having their uncombined carbon in nodular form may be prepared by introducing certain treating agents into a molten bath, such as cerium and magnesium. But the practice of the prior art processes involves certain difficulties; and such processes have not proved entirely satisfactory for large scale commercial production. For example, the introduction of magnesium into molten metal is an extremely difficult operation, primarily because of its relatively low boiling point (1107° C.) and high degree of reactivity. Its introduction into a molten bath in the usual way produces a violent reaction, which makes the operation hazardous. Such violence causes relatively high and unpredictable magnesium losses so that reproducibility of a uniform nodular cast iron with the same composition is virtually impossible.

Numerous attempts have been made to minimize or eliminate these difficulties by alloying elemental magnesium with other substances, for example nickel and copper. But even these magnesium alloys have certain objectionable features. For example, undesirable chilling of the molten iron occurs when large quantities of alloys are added thereto; the alloys are expensive; the properties of the cast iron product may be adversely affected by one or more elements alloyed with magnesium; and some of the alloying substances are not eliminated by remelting so that the scrap may contain intolerable amounts of such materials.

In the copending application of James W. Estes and Grant E. Spangler, Treating Molten Iron, Serial No. 486,714 (assigned to the assignee of the present application), there is disclosed and claimed an improved method for preparing an ungraded and nodular gray cast iron. In the practice of such method, an inert gas stream is passed into the molten metal beneath its surface. A mixture of finely divided calcium carbide particles and finely divided magnesium particles is fed into this gas stream, the magnesium particles constituting about 5% to 15% by weight of the mixture. In certain instances, however, it has been found desirable to include magnesium in amounts exceeding 15% of the mixture in order to obtain the desired nodular cast iron. In such respect, the process of the copending application does not completely and adequately meet the demands of the cast iron industry. The present invention constitutes a further improvement of the process disclosed in the above-identified copending application.

The primary object of the present invention is to provide an improved method, adapted for large scale commercial use, for introducing calcium carbide and elemen-

2

tal magnesium beneath the surface of molten metal, to produce a nodular cast iron product having improved physical and mechanical properties.

Another object is to provide an improved method for injecting finely divided particles of calcium carbide and magnesium, particularly when the magnesium particles exceed 15% by weight of the total mixture or solids.

A further object of the present invention is to provide an improved method for injecting calcium carbide and relatively large quantities of magnesium into molten metal at normal founding temperatures without any injection failures caused by plugging and similar factors.

A still further object is to provide a novel addition agent particularly adapted to introduce calcium carbide and varying amounts of magnesium into cast iron for treatment thereof, resulting in a cast iron product having its graphite in nodular or spheroidal form.

These and other objects and advantages of the present invention will become more apparent from the following detailed description of the invention.

Broadly stated, the treating agent of the invention is a mixture of finely divided particles of calcium carbide, magnesium chips, and a relatively small quantity of calcium oxide. The calcium oxide is admixed with the magnesium chips prior to mixing with the calcium carbide. The invention further contemplates an improved process for treating molten ferrous baths, particularly gray cast iron baths, with the novel treating agent to effectively introduce and incorporate magnesium in said baths, to reduce the sulphur content thereof, and to provide gray cast irons having its graphite in nodular form.

In its preferred embodiments, the agent contains about 5% to about 20% magnesium, about 2% to about 10% calcium oxide, and the balance essentially calcium carbide. Very good results are obtained when the amount of calcium oxide is about one-half that of the magnesium.

Generally speaking, the invention comprises establishing a molten bath having a gray cast iron composition, injecting a relatively dense stream of inert gas and a mixture comprising calcium carbide, magnesium, and calcium oxide beneath the surface of the metal, and then promptly casting the iron. Such composition contains more than 90% iron, carbon from 1.7% to 4.5%, and silicon from 1.0% to 3.5%. Other elements conventionally found in cast irons are present, such as sulphur, manganese and phosphorous in usual amounts, and impurities or traces of other elements such as titanium and zirconium. Suitable apparatus for injecting the treating agent include, for example, the screw feeding device shown in Hulme Patent No. 2,577,764; the batch feeder disclosed in the copending United States patent application Serial No. 430,864, now abandoned; or the fluidizer injection device shown in the copending United States patent application Serial No. 324,998 (all assigned to the assignee of the present application). All of these apparatus are adapted for feeding a solid-gas stream having an apparent density of about one-quarter to two cubic feet of gas per pound of solids. For purposes of this invention, various inert gases may be used provided they do not enter into any chemical or oxidizing reaction with the molten metal or treating agent. Dry nitrogen could be employed, for example, since it is readily available and inexpensive. However, other gases which can be used and are just as efficient as nitrogen are helium, argon and carbon dioxide.

For best results, the treating agent contains about 5% to 20% magnesium and 2% to 10% calcium oxide, and the balance calcium carbide. The amount of calcium oxide is preferably about one-half that of magnesium. The presence of a critical amount of calcium oxide in the mixture prevents or minimizes plugging of the injection tube. In the initial tests made with respect

to treatment of molten metals with an agent containing magnesium, it was readily apparent that the prevention of tube plugging was a serious problem, independent of the hazards ordinarily involved and independent of the efficiency of treatment. It was noted that with treating agents composed of only magnesium and calcium carbide, incidence of injection failures by reason of tube plugging increased as the magnesium content of the calcium carbide-magnesium mixture exceeded 10%; and that evidence of injection failures approached 100% as the magnesium content of such mixture approached 20%. Although the theoretical explanation is not fully understood, it is believed that as the percentage of magnesium increases, the possibilities of contact between the particles of magnesium also increase, and consequently, any melting of magnesium particles where physical contact has been established would cause agglomeration in the tube, and a plug would result. But when the treating agent includes lime in amounts described above, trouble-free injections of mixtures containing as high as 20% magnesium have been made. When the percentage of calcium oxide is more than about one-half the magnesium content, the oxide tends in a sense to coat the magnesium mechanically and thus prevent intimate reaction of the magnesium with the molten metal, so that the amount of graphite appearing in nodular form is significantly reduced.

The amount of magnesium injected is preferably about one to six pounds of magnesium per ton of iron, and the amount of calcium oxide injected is thus preferably about one-half to three pounds per ton of molten metal. The amount of calcium carbide injected will depend upon the amount of certain undesirable impurities in the molten iron, such as sulphur and oxygen. The higher the content of such impurities in the untreated molten metal, the greater should be the amount of carbide injected. Since desulphurization is required in most instances, it is preferred to inject finely divided calcium carbide beneath the surface of the metal to reduce the sulphur content thereof from a relatively high level to a relatively low level, e.g., to a level of 0.03% or less, and preferably to about 0.01%, and thereafter injecting the treating agent in an amount sufficient to produce the desired nodular cast iron. In some instances, it is also preferred to inoculate the molten metal with a conventional graphitizing agent such as ferrosilicon subsequent to the injection of the agent and prior to casting.

For purposes of the present invention, the apparent density of the gas-solid stream at the point of its introduction into the molten metal will range from one-quarter to about two cubic feet of gas per pound of solids. The gas is maintained at a pressure sufficient to

overcome the static head of molten iron and thus prevent the entrance of metal into the passage through which the mixture is injected. The rate of feeding will vary depending upon the size of the metal container and

5 the type of injection apparatus.

The treating agent of this invention is prepared by intimately mixing by any conventional means preferably about 5 to 20 parts of magnesium powder and about 2 to 10 parts of calcium oxide, which admixture is then 10 mixed with about 93 to 70 parts finely-divided calcium carbide. The calcium carbide may be a commercial grade of calcium carbide, quite free of impurities, as made in electric arc furnaces, from calcium oxide and high quality coke. The carbide particles pass through 15 a 20-mesh screen, and about 90% of the particles are retained on a 200-mesh screen. The magnesium particles pass through a 20-mesh Tyler standard screen, and about 90% of the particles will be retained on a 100-mesh screen. Examined under a microscope, these particles have irregular edges which are frequently rolled 20 up. The quantities of the various components of the novel treating agent used per ton of gray cast iron range between 10 and 18 pounds of calcium carbide, between  $\frac{1}{2}$  and 12 pounds of magnesium, and between  $\frac{1}{4}$  and 6 25 pounds of calcium oxide. In any event, the magnesium content should not exceed 20% of the total mixture.

The following table includes examples of hypo-eutectic and hyper-eutectic cast irons, their compositions, and properties after treatment. The composition of the metal 30 in the molten bath is that used to make a conventional gray cast iron. In the examples, the iron constitutes more than 90%, the carbon from 3.30 to 3.60%, and the silicon from 1.40% to 1.90%. Desulphurizing and benefiting such as deoxidation, was first effected by the injection of 35 calcium carbide alone, in a proportional amount of 16 pounds of carbide per ton of molten metal. With this first step, the sulfur level of the iron is reduced to less than 0.03%, and the iron is more receptive to the beneficial effects of magnesium. Immediately thereafter, the cast 40 irons were treated with a reagent comprising (1) calcium carbide, magnesium, and lime, or (2) calcium carbide, magnesium, lime, and a rare earth oxide. A small amount of a rare earth oxide (REO) may be incorporated in the carbide-magnesium-lime mixture to insure a totally 45 nodular cast iron. The REO contains about 50% cerium oxide, 20% lanthanum oxide, and the balance consists of other rare earth substances. In the practice of the present invention, the REO is finely divided, being at least 20 by 0 mesh size. The tables show the proportioning of the various constituents of the treating agent, the compositions and the physical properties of the treated metal, when carbide treatment is first effected.

Table I

| Sample No. | Injection Mix (Lbs./Ton) |       |      |      | Percent Late FeSi | Chemical Analyses |      |      |        |                    |       |       |       | Properties |        |        | Chill Depth (1/32") |
|------------|--------------------------|-------|------|------|-------------------|-------------------|------|------|--------|--------------------|-------|-------|-------|------------|--------|--------|---------------------|
|            | CaC <sub>2</sub>         | REO   | Mg   | CaO  |                   | T. C.             | Si   | Mn   | Base S | Final S            | P     | Mg    | C. E. | U.T.S.     | B.H.N. | Elong. |                     |
| 894-1----- | 20                       | 1.0   | 3.0  | 1.5  | 1.00              | 3.55              | 2.47 | 0.35 | 0.093  | <sup>1</sup> N. R. | 0.037 | 0.028 | 4.37  | 66,900     | 154    | 19.5   | 20                  |
| 896-1----- | 13                       | 1.0   | 4.0  | 2.0  | 1.00              | 3.59              | 2.22 | 0.34 | 0.103  | N. R.              | 0.032 | 0.038 | 4.33  | 66,500     | 152    | 18.0   | 22                  |
| 897-1----- | 17                       | ----- | 2.4  | 1.2  | 1.00              | 3.41              | 2.52 | 0.33 | 0.085  | N. R.              | 0.042 | N. R. | 4.25  | 47,900     | 150    | 4.0    | 36                  |
| 898-1----- | 21                       | ----- | 3.0  | 1.5  | 1.00              | 3.44              | 2.45 | 0.34 | 0.098  | N. R.              | 0.042 | N. R. | 4.26  | 53,850     | 152    | 5.5    | 24                  |
| 899-1----- | 21                       | ----- | 3.0  | 1.5  | 1.00              | 3.55              | 2.40 | 0.34 | 0.096  | N. R.              | 0.035 | N. R. | 4.35  | 65,300     | 159    | 13.5   | 23                  |
| 900-1----- | 16                       | 1.0   | 2.0  | 1.0  | 1.00              | 3.53              | 2.49 | 0.72 | 0.091  | N. R.              | 0.044 | N. R. | 4.36  | 60,100     | 166    | 4.5    | 15                  |
| 905-1----- | 20                       | 1.0   | 3.0  | 1.5  | 1.00              | 3.56              | 2.45 | 0.62 | 0.103  | 0.006              | 0.035 | N. R. | 4.38  | 76,900     | 181    | 7.0    | 24                  |
| 906-1----- | 62                       | 2.0   | 12.0 | 4.0  | 1.00              | 3.54              | 2.37 | 0.33 | 0.107  | 0.004              | 0.034 | 0.088 | 4.33  | 91,800     | 198    | 9.5    | 44                  |
| 907-1----- | 15                       | 1.0   | 1.0  | 0.5  | 1.00              | 3.46              | 2.54 | 0.71 | 0.102  | 0.012              | 0.038 | 0.008 | 4.31  | 49,200     | 148    | 2.5    | 22                  |
| 908-1----- | 16                       | ----- | 1.0  | 0.5  | 1.00              | 3.51              | 2.51 | 0.72 | 0.090  | 0.014              | 0.035 | N. R. | 4.35  | 22,800     | 113    | 1.0    | 16                  |
| 909-1----- | 15                       | 1.0   | 1.0  | 0.5  | 1.00              | 3.68              | 3.10 | 0.17 | 0.108  | N. R.              | 0.047 | N. R. | 4.73  | 53,300     | 144    | 4.5    | 7                   |
| 911-1----- | 10.8                     | 0.51  | 2.05 | 0.25 | 1.00              | 3.30              | 2.21 | 0.74 | 0.103  | N. R.              | 0.089 | N. R. | 4.07  | 65,500     | 185    | 3.0    | 32                  |
| 912-1----- | 20                       | 1.0   | 4.0  | 2.0  | 1.00              | 3.47              | 2.23 | 0.76 | 0.115  | N. R.              | 0.083 | N. R. | 4.24  | 92,800     | 212    | 5.0    | 32                  |
| 913-1----- | 20                       | 1.0   | 4.0  | 2.0  | 1.00              | 3.38              | 2.15 | 0.72 | 0.103  | N. R.              | 0.075 | N. R. | 4.09  | 99,200     | 232    | 4.5    | 33                  |
| 914-1----- | 15                       | 1.0   | 1.0  | 0.5  | 1.00              | 3.34              | 2.14 | 0.74 | 0.103  | N. R.              | 0.075 | N. R. | 4.07  | 59,300     | 174    | 2.5    | 32                  |
| 915-1----- | 16                       | ----- | 1.0  | 0.5  | 1.00              | 3.34              | 2.17 | 0.74 | 0.101  | N. R.              | 0.021 | N. R. | 4.10  | 45,650     | 185    | 1.0    | 18                  |
| 888-1----- | 34                       | 2.0   | 4.0  | 4    | 1.00              | 3.61              | 2.25 | 0.32 | 0.106  | N. R.              | 0.032 | 0.024 | 4.36  | 64,700     | 159    | 7.5    | 18                  |
| 890-1----- | 32                       | 2.0   | 4.0  | 2    | 1.00              | 3.57              | 2.46 | 0.33 | 0.089  | N. R.              | 0.035 | 0.036 | 4.39  | 67,200     | 152    | 19.5   | 20                  |
| 891-1----- | 20                       | 1.0   | 3.0  | 1.5  | 1.00              | 3.48              | 2.46 | 0.34 | 0.084  | N. R.              | 0.024 | 0.032 | 4.30  | 70,850     | 166    | 14.0   | 20                  |

<sup>1</sup> Not requested.

The phrase, Percent Late FeSi, refers to the addition of ferrosilicon (75% silicon) as a percentage of the iron being treated. The ferrosilicon was added by reladdling, although it may be injected with a carrier gas. The data under the heading "Chemical Analyses" refers to the analyses of the treated metal with respect to silicon, manganese, and phosphorus; initial and final sulfur contents; the total carbon content and carbon equivalent referred to as T. C. and C. E., respectively; and the retained magnesium content. The Injection Mix data defines the amount of materials injected in terms of pounds of each material per ton of iron. The properties shown include ultimate tensile strength (U. T. S.), Brinell hardness number (B. H. N.), and elongations (Elong.) as percentages in two inches. The chill figure was obtained by casting into a sand mold against a graphite block as a base. The wedge formed was 3½ inches high, ¾ inch wide at the top and ⅜ inch at the bottom. The tabulated figures are the depths of the chill from the bottom of the wedge contacting the block in 32nds of an inch.

In all the examples set forth in the above table, the treating agent includes a small amount of powdered lime (CaO). Ordinarily, the lime was added in fine powdered form to the various mixtures which may be mechanically mixed, for example, by tumbling. Best results, mechanically and metallurgically, were obtained when the powdered lime was added in an amount equal to one-half the amount of powdered magnesium by weight in the mixture. In no instance did plugging occur in the injection tube when the lime content varied from 25% to 50% of the magnesium content. Further, the use of the lime particles did not adversely affect the carbide-magnesium treatment, as evidenced by the physical properties of the metal treated. For example, the tensile strengths of the cast irons treated in accordance with the process of the present invention range from about 50,000 to 99,000 p. s. i. The addition of lime to the various mixtures permitted the use of 10%–15% magnesium concentration by weight and even to as high as 20% without any occurrence of plugging in the injection tube. It is believed that the lime coats the particles of magnesium powder and the injection tube wall, thus preventing melting or sintering of the particles to the tube or to each other. Optimum flow results were obtained when the lime particles were finer than 100 mesh. The lime used in the examples is a soft light grade of technical calcium oxide which contains considerable quantities of calcium carbonate and calcium hydroxide. The lime used in the examples has the following analyses:

| CaO                      | Percent<br>Ca(OH) <sub>2</sub> | Percent<br>CaCO <sub>3</sub> | Percent<br>CaO |
|--------------------------|--------------------------------|------------------------------|----------------|
| as received.....         | 56.8                           | 2.5                          | balance.       |
| crushed and roasted..... | 1.5                            | 11.9                         | balance.       |

The lime described above has a tendency to adhere to the smooth surfaces of the injection tube, and thus prevent or minimize melting or fusing of the treating particles to the walls of the tube. The lime provides lubricating properties to the addition agent of the invention, that is, to mixtures comprising at least finely-divided calcium carbide and magnesium. The lime also serves to maintain a flow of solids having a substantially uniform composition of solids, through the entire treating operation.

It will be noted from the examples listed above that the presence of the lime powder in the treating mixture did not adversely affect the properties of the resulting product when the treating mixture comprises (1) calcium carbide, magnesium, and lime, or (2) calcium carbide, magnesium, rare earth oxides, and lime. When the carbide content of the treating agent was maintained constant and the magnesium content was increased, the properties of the as cast product were improved; and when rare earth oxides were added to the mixture, the

properties were improved, as would be expected in view of the prior art.

It will now be appreciated that the instant invention provides a practical method for treating molten iron compositions with addition agents comprising calcium carbide and magnesium in an amount as high as twenty (20) percent by weight. The amount of lime added to the mixture is preferably 20% to 50% of the magnesium. With the use of the novel agent, plugging in the injection tube is virtually eliminated.

It will be understood that the invention is not limited to the specific examples described herein, but may be practiced in other ways without departing from the spirit and scope of the invention as defined in the following claims.

What we claim is:

1. A method of improving the physical properties of an as-cast gray cast iron comprising establishing a molten quantity of gray cast iron containing more than 0.03% sulphur, injecting into said molten cast iron sufficient calcium carbide so that the quantity of the sulphur is reduced to less than about 0.03% sulphur, injecting a mixture comprising about 5% to 20% magnesium chips, 2.0% to 10% calcium oxide, and 70% to 93.0% finely divided calcium carbide, said mixture being carried beneath the surface of the molten iron by an inert gas, and the stream of gas and mixture containing from about ¼ to 2 cubic feet of gas per pound of solids injected.
2. A method according to claim 1, in which the amount of calcium oxide in said mixture is about one-half that of magnesium.
3. A method according to claim 1, in which a finely divided oxide is incorporated in said mixture, and the amount of said last mentioned oxide employed is about 1 to 2 pounds per ton of molten iron.
4. A method for the production of nodular cast iron comprising establishing a molten gray iron composition containing more than 90% iron, carbon from 1.7% to 4.5%, silicon from 1.0% to 3.5%, and sulfur in excess of 0.03%, incorporating into said bath a treating agent containing about 5% to 20% magnesium, about 2.0% to 10% calcium oxide, and about 70% to 93% finely divided calcium carbide, said agent being injected into said molten iron with an inert gas carrier, in the ratio of from about ¼ to 2 cubic feet of gas per pound of solids injected, the amount of calcium carbide employed being in excess of that required to reduce the sulphur content to about 0.01%, and casting said iron composition to form castings characterized by the occurrence of uncombined graphite in predominantly nodular form.

5. A method for the production of nodular cast iron comprising establishing a molten gray iron composition containing more than 0.03% sulfur, injecting into said molten iron sufficient calcium carbide to reduce the sulfur content to less than 0.03%, injecting beneath the surface of said molten metal by means of a carrier gas a treating agent comprising about 5% to 20% magnesium, 2.0% to 10% calcium oxide, and the balance finely divided calcium carbide, inoculating said treated iron with a conventional graphitizing agent subsequent to injection of said agent and prior to casting, and casting said iron composition promptly to form castings characterized by the presence of uncombined graphite in predominantly nodular form.

6. A homogeneous treating material particularly adapted for introducing magnesium into molten gray cast iron with very little loss, said material containing about 5% to 20% of small chip-like particles of elemental magnesium, about 2% to 10% calcium oxide, and about 70% to 93% calcium carbide, said oxide and carbide particles being in finely divided form.

7. An agent particularly adapted for the production of nodular cast iron, said agent containing about 5% to 20% magnesium, calcium oxide in an amount sufficient to prevent any significant loss of magnesium prior to its

introduction into molten metal, and the balance substantially calcium carbide, said magnesium particles being of a fineness sufficient to pass through a 20 mesh screen but which particles will be retained on a 100 mesh screen, and said calcium carbide particles being of a fineness sufficient to pass through a 20 mesh screen but which will be retained on a 200 mesh screen, said magnesium and calcium oxide particles being thoroughly mixed.

8. A homogeneous treating material particularly adapted for continuously injecting magnesium into a molten gray cast iron with very little loss, said material containing about 5% to 20% of small chip-like particles of elemental magnesium, an amount of calcium oxide particles equal to about one-half that of magnesium, and the balance substantially finely divided particles of calcium carbide, said magnesium and calcium oxide particles being thoroughly mixed.

9. The treating material as defined in claim 8 and being further characterized in containing finely divided rare earth oxide, the amount of said last-named oxide employed being about 1 to 2 pounds per ton of molten iron treated.

10. A homogeneous particulate treating material particularly adapted for introducing magnesium into a molten ferrous metal composition, comprising magnesium, calcium oxide and calcium carbide, the magnesium being present in an amount up to 20%, the calcium oxide being present in the amount of about 2% to 10% and the balance being substantially calcium carbide.

11. A homogeneous particulate treating material particularly adapted for introducing magnesium into a molten ferrous metal composition, comprising magnesium, calcium oxide and calcium carbide, the magnesium being present in an amount up to 20%, the calcium oxide being present in an amount equal to about 20% to 50% of the amount of magnesium, and the balance being substantially calcium carbide.

References Cited in the file of this patent

FOREIGN PATENTS

|    |         |         |                |
|----|---------|---------|----------------|
| 20 | 514,115 | Belgium | Sept. 30, 1952 |
|    | 177,794 | Austria | Mar. 10, 1954  |